

# UNITED STATES PATENT OFFICE

WALTER G. CORNELIUS, OF PIRU, CALIFORNIA

## TREE PAINT

No Drawing.

Application filed September 22, 1924. Serial No. 739,200.

The object of my invention is the production of a composition or paint to be applied to cuts, wounds, bruises and all exposed wood surfaces of trees and shrubbery made by accidents—pruning, tree-surgery or treating diseases.

My composition consists of a mixture of gilsonite,—coal-tar,—rosin and gasoline.

In preparing the composition I prefer to use the ingredients in about the following proportions viz: fifty pounds gilsonite—ten pounds rosin—ten gallons coal tar—and four gallons of gasoline or benzine. Very good results may be obtained, however, when the ingredients are varied in a small amount either way.

These ingredients are mixed in the following manner: The gilsonite and rosin are put in one container. The coal tar in another. Both are heated until thoroughly melted and boiling. The coal tar is then added to the mixture—stirred thoroughly—put in cans and set away to cool. When cold the composition is too thick for use, but is thinned with gasoline or benzine, as wanted and applied cold.

My composition is water proof, is weather proof, adheres without cracking when it dries to the surface to which it is applied, and is very efficient in all respects as it helps nature to heal and cover all wounds for which it is made.

I claim—

1. A tree paint consisting of fifty pounds of gilsonite, ten pounds of rosin, ten gallons of coal tar and four gallons of gasoline.
2. A tree paint consisting of a mixture of gilsonite, coal-tar, rosin and gasoline substantially in the proportions set forth.

WALTER G. CORNELIUS.